

May 10, 1949.

W. J. SWEENEY

2,469,751

COLD STARTING MOTOR FUEL

Filed Sept. 1, 1943

2 Sheets-Sheet 1



FIG. -1

William J. Sweeney Inventor

By Ph. Young Attorney

May 10, 1949.

W. J. SWEENEY

2,469,751

COLD STARTING MOTOR FUEL

Filed Sept. 1, 1943

2 Sheets-Sheet 2



FIG.-2

William J. Sweeney Inventor

By Ph. Young Attorney

## UNITED STATES PATENT OFFICE

2,469,751

## COLD STARTING MOTOR FUEL

William J. Sweeney, Summit, N. J., assignor to  
 Standard Oil Development Company, a corporation of Delaware

Application September 1, 1943, Serial No. 500,754

2 Claims. (Cl. 44—52)

1

The present invention relates to an improved method for starting gasoline engines at low temperatures and to a priming fuel especially adapted for the process. The invention will be fully understood from the following description and the drawings.

Fig. 1 is a diagrammatic plan of the equipment required for starting the engine at low temperature by the present method, and

Fig. 2 shows distillation curves of several fuels made up according to the invention and indicates their characteristics.

Everyone who has operated a motor car in cold weather knows the increased difficulties of starting the engine at progressively lower atmospheric temperature. With airplanes these difficulties are perhaps even greater since it is frequently necessary to start motors at temperatures far below those at which automobiles are apt to be operated. For example, it is a common occurrence in some localities to encounter atmospheric temperatures of  $-20^{\circ}$ ,  $-30^{\circ}$  or even  $-65^{\circ}$ , and it is desirable to have some general method, fuel and procedure which is capable of starting engines at these low temperatures, and particularly a method and particular fuel which can be successfully used over this entire range of temperature without variation.

The starting of cold motors is an old problem and long ago it was proposed that special priming fuels be employed, that is to say, that the engine be started on a special fuel, generally lighter and lower boiling than the ordinary operating fuel. Such attempts have not, however, been successful, particularly at the very low temperatures far below zero. One reason for this lack of success lay in the nature of the particular fuels that were used and, secondly, in the method in which they were employed.

Prior priming fuels have in almost every case consisted of extremely narrow range cuts of light petroleum hydrocarbons, in many cases pure hydrocarbons, principally propane, butane and the like. On the contrary it has now been found that the fuel best suited for this purpose is a relatively wide cut mixture of several volatile hydrocarbons of different boiling points. The prior methods have depended either on the direct discontinuous injection of a choking stream of fuel or on the application of the priming fuel just as the operating fuel was used, that is to say, it was evaporated into the air stream and was carried into the engine along with and roughly proportional to the amount of air fed. In contrast, the present method consists of continuously

5

10

15

20

25

30

35

40

45

50

55

2

forcing a stream of liquid fuel into the intake manifold quite independently of the air stream and the fuel is so composed that it is vaporized in such an amount that the vaporized quantity always forms an explosive mixture with air. Any excess remains as liquid and is removed in this form without combustion. Thus the method depends on the continuous feeding of an excess of liquid fuel during the entire starting period so that the amount vaporized always forms a combustible mixture under the entire range of starting conditions.

Referring to the drawing, Fig. 1 is a diagrammatic plan of the equipment required for the present process. Numeral 1 denotes a storage tank for the priming fuel which will be described for the present as a wide cut mixture of normally gaseous and low boiling hydrocarbons. The supply tank need not be described in detail and it will suffice to say that it is of any type suitable for the storage of very volatile products which may have a Reid vapor pressure of 40 to 75 pounds per square inch. The fuel is drawn in liquid condition through the line 2 by the fuel pump 3 and a by-pass line is provided around the pump and fitted with a valve 4, so that the pump may be operated at a constant speed, and by adjusting the valves 2' in the feed line 2 and valve 4 in the by-pass line, it is possible to deliver an adjusted amount of fuel to the engine while the pump is operating at a constant speed. The fuel line 2 discharges the liquid fuel into the engine manifold 5 at any convenient point, preferably at the entrance of the supercharger which is indicated at 6. A suitable cranking device is shown at 7 and the ignition switches at 8. The operating fuel tank is number 10 and the ordinary fuel is withdrawn by the pipe 11 which contains the valve 12 and the fuel pump 13. The fuel pump has a by-pass line 13' similar to that supplied with the priming fuel pump so that this pump may be operated at a constant speed without delivering any fuel to the engine when the valve 12 is closed and 13' is opened. This fuel is injected into the engine at 14, while the air enters in the usual way at 15, and is measured by the carburetor 16 which discharges in the usual manner into the intake manifold 5.

In the operation of the present process, the engine will naturally be at atmospheric temperature and the priming fuel pump 3 is started with valves 2' and 4 being adjusted so that the desired volume of fuel is forced at a pump pressure of 2 to 50 pounds through the line 2 and into the

engine manifold. The amount of fuel supplied should be calculated so as to be sufficient to operate the engine under idling conditions, with a slight excess, say 5 to 10%. It will be understood that the operating fuel pump 13 is also set in motion, but the valve 12 is closed so that none of the operating fuel is delivered to the engine. The engine is now spun by the use of the cranking device 7 and when the engine speed reaches a proper value, the switch 9 is closed so that the priming fuel is ignited and the engine starts. The speed at which the engine must be spun cannot be specified with exactness since it is primarily a function of the particular engine, its design and construction, and the lubricants used, but in general it will be of the order of 50 R. P. M.

The priming fuel is allowed to flow for several seconds before the switch 9 is closed, and even after ignition, it is desirable to operate the engine on the priming fuel for 30 to 120 seconds in order to warm up the engine. At the end of this time, valve 2' is closed and the valve 12 is opened simultaneously so that the operating fuel is substituted for the priming fuel.

The various operations indicated before may be effected by hand or mechanically and with the proper fuel it has been found that various types of engines can be consistently started at temperatures over the range of -65° to +20° F. easily and quickly. Slight variations in the operation may be desirable, depending on the particular engines, just as indicated above, where desired rotational speed of the engine may be varied and in the same manner the amount of fuel required is also variable.

From what has been said, it will be appreciated that the composition of the priming fuel is a most important feature in the present invention and the success of the method depends on the use of a fuel consisting of a liquid mixture of several normally gaseous and liquid hydrocarbons, ranging from 3 to 8 carbon atoms, and having a wide boiling range, that is to say, a boiling range of at least 75 Fahrenheit degrees between the 10% and 90% distillation points. It is preferable to provide even a greater spread than this, for example 100 or even 150 Fahrenheit degrees.

The fuel must contain a sufficient amount of very volatile constituents, which will be vaporized at the lowest starting temperature likely to be encountered. In addition to these fractions, there must also be intermediate constituents boiling between the low boiling initial fractions and the volatile fractions of the operating fuel. Such fractions serve to fill the gap between the starting fractions and the operating fuel. It will be understood that the proportions of these various light, intermediate fractions are of extremely great importance. If the quantity of the lighter fractions is too great, there would be difficulties in starting at temperatures from -20° to +20° F., and also there is a considerable tendency to vapor locking at these temperatures. Storage and handling difficulties are also increased. If, on the other hand, an insufficient quantity of these materials is provided, the fuel will fail to start at the very low temperatures. It is particularly important that there should be, as stated before, a wide boiling range in the fuel.

As to the actual composition of the fuel, it is made up principally of the hydrocarbons from propane to octane and it is preferred to use a substantial quantity of the iso compounds be-

cause of their superior anti-detonation quality. Ethane or ethylene are not absolutely required, although it is desirable to provide from 2 to 3% by volume and not more than about 5%. The amount of propane and propylene, that is to say, C<sub>3</sub> hydrocarbons, will vary between about 10 and 25%. The butanes, C<sub>4</sub> fractions, vary from about 15 to 45% and the pentanes, C<sub>5</sub> fractions, from 30 to 40%. In addition to the C<sub>3</sub> through C<sub>5</sub> fractions, it is also preferable to add a certain amount of the heavier components which may be selected from the hexanes, heptanes and octanes. This is preferably in from 10 to 25% of the final fuel mixture and instead of these pure compounds, if desired, ordinary gasoline can be added or, if preferred, aviation gasoline which supplies these heavier components.

The above percentages may be looked upon as limits and it will be understood that the fuel is thus balanced so as to give a smooth boiling curve which has the following characteristics:

|                        | Max. | Min. |
|------------------------|------|------|
| 25                     | °F.  | °F.  |
| 10% Evaporated at..... | +30  | -30  |
| 50% Evaporated at..... | +100 | +50  |
| 90% Evaporated at..... | +170 | +100 |

It will be understood that olefins may be used instead of paraffins or mixtures of olefins and paraffins may be used and various fuel ingredients may be added also, such as top lubricants, anti-detonation agents, inhibitors and the like, just as in any other fuel.

In further explanation of the present method, it may be said that an engine must be operated on a mixture of vaporized fuel and air in which the proportion of fuel to air, that is to say, the air-fuel ratio, must be at all times within the explosive limits. These limits are definite characteristics of the fuel itself and are such that a mixture may be too lean or too rich for ignition. In the usual method of operating gasoline engines, the fuel is vaporized in the inlet air and most prior attempts to solve the low temperature starting problem have supplied the fuel with the air in the usual manner, that is to say, the flow of air controlling the flow of fuel either by evaporation or mechanically. If a pure hydrocarbon, such as propane or butane is used, the explosive limits of the mixture are quite narrow, of the order of 20 to 25 Fahrenheit degrees, and it is very difficult, practically impossible, in the ordinary method of operation to keep the mixture constantly within this narrow range, where explosion is possible. When prior priming fuel vaporizes, there is a drop in temperature and this is frequently enough to bring the mixture out of the explosive range. Furthermore, when an engine starts, its speed rapidly increases and its temperature also rises, which makes it almost impossible to adjust the volume of fuel to air so as to hold the fuel-air mixture within the narrow explosive range within the very short time available to the operator. No simple mechanical device has been found to accomplish this desired result. In other words, the changes in temperature and other conditions are so rapid during the starting period that it is impossible for an operator to maintain the mixture constantly within the explosive range and the air volume is not a suitable control means by which the requisite amount of fuel can be provided at all times. This is thought to be the reason for the sputtering and stalling which is so gener-

ally met in attempting to start an engine at low temperatures. In the present invention, these faults are corrected first by feeding the fuel, independent of the air, constantly and at a rate sufficient for the operation of the engine under the starting conditions or slightly in excess thereof. The fuel is fed as a liquid and not along with the air in vaporized condition. Thus a considerable volume of fuel is constantly being supplied and is always available to be vaporized as needed. Some of the priming fuel, especially at low temperatures before the engine is warmed up, will not be vaporized at all and will be discharged from the engine as a liquid unburned but the important point is that as the engine speed is increased and as the temperature rises, sufficient fuel is always present for vaporization as required. The second important point to be understood is that the fuel itself being a wide cut rather than a very narrow cut, is characterized by a wide range of explosive limits rather than narrow explosive limits. For example, instead of the 20 to 25° characteristic of a pure hydrocarbon of the lower range, the present mixtures have ranges in excess of 100 Fahrenheit degrees, and preferably of 200, 250 or even 300 Fahrenheit degrees. This permits a wider range of possible operation and the sputtering and stalling is then practically eliminated, since sufficient time is given for adjustment within the explosive range. From the above it will be apparent that the present method requires the particular fuel, or in other words, the composition of the priming fuel is a feature of the method itself.

As examples of the types of priming fuels, the following may be considered typical:

*Example 1*

|                 | Percent By Volume | Percent By Weight |
|-----------------|-------------------|-------------------|
| Propane.....    | 12.2              | 10.3              |
| Isobutane.....  | 19.0              | 18.0              |
| N-butane.....   | 18.6              | 18.0              |
| Isopentane..... | 15.8              | 16.8              |
| N-pentane.....  | 16.0              | 16.8              |
| Neohexane.....  | 18.4              | 20.1              |

This fuel had a Reid vapor pressure of 56.5 pounds and was quite satisfactory over a wide range from -60° F. to +200° F. The boiling range has been plotted in Fig. 2, as fuel #1.

*Example 2*

|                 | Percent By Volume | Percent By Weight |
|-----------------|-------------------|-------------------|
| Propane.....    | 20.0              | 17.1              |
| Isobutane.....  | 14.4              | 13.5              |
| N-butane.....   | 14.0              | 13.5              |
| Isopentane..... | 31.6              | 33.6              |
| N-pentane.....  | 12.4              | 13.4              |
| Neohexane.....  | 7.6               | 8.9               |

The Reid vapor pressure of this fuel was 69 1/4 pounds. It was also quite satisfactory at low temperatures but had a tendency to vapor lock at 0° F. to 20° F. Its distillation curve is also plotted in Fig. 2. These distillations are carried out with a fluid immersed in a mixture of alcohol and dry ice condensed in the same manner, the temperature being recorded in the same manner as is familiar in the Engler distillation procedure. This fuel was distilled twice on successive days and both curves are plotted in Fig. 2 as

75

fuel #2 and #2a, in order to indicate the degree of reproducibility.

*Example 3*

5 The fuel of this example was made by adding to an aviation gasoline certain low boiling hydrocarbons.

|                           | Percent By Volume | Percent By Weight |
|---------------------------|-------------------|-------------------|
| 10 Propane.....           | 20                | 17.0              |
| Isobutane.....            | 28.2              | 27.0              |
| N-butane.....             | 34.5              | 36.0              |
| Isopentane.....           |                   |                   |
| N-pentane.....            |                   |                   |
| 15 Aviation Gasoline..... | 17.3              | 20                |

The aviation gasoline had the following characteristics:

20 Gravity A. P. I. ..... degrees 68.8

Reid V. P. ..... 6.1

ASTM distillation:

|           |         |
|-----------|---------|
| 25 10% at | °F. 140 |
| 50% at    | °F. 158 |
| 90% at    | °F. 178 |
| Final     | °F. 199 |

This complete fuel had a Reid vapor pressure of 65 1/2 pounds. In tests with this fuel, a Wright engine, type G-2600, was started successfully and consistently at the following temperatures: -20° F., -40° F., -50° F., -55° F., -60° F. and -65° F. The fuel was fed independent of the air at a pressure of about 10 pounds per square inch.

35 The spark timing was about 20° before top center and throttle setting was 9° from the horizontal closed position. Cranking speed was 50 R. P. M. and the fuel was fed into the air line just at the entrance of the supercharger. The 40 feeding of the priming fuel was continued for from 30 to 120 seconds after the engine took hold, before the ordinary operating fuel was substituted for the priming fuel. This was accomplished easily and smoothly. The operation was 45 marked by the absence of false starts, sputtering and stalling.

From the above description, it will be understood that many minor changes in the fuel are possible within the ranges given. Certain 50 hydrocarbons may be eliminated altogether without pronounced ill effect. For example, hexane is absent in the fuel of Example 2, but it is believed best to include in all fuels propane, butane and pentane and some of the higher hydrocarbons which may be selected from the group of hexane, heptane and octane or, better, to use a portion of gasoline, say an aviation gasoline which will contain these several hydrocarbons. As stated before, ethane is not necessary but up to 5% may be included and it is of assistance in starting when the extremely low temperatures are encountered.

I claim:

1. A priming fuel for starting gasoline engines 65 at low temperatures comprising a liquid mixture of normally gaseous and low boiling paraffinic hydrocarbons, 10% to 25% having 3 carbon atoms, 15% to 45% having 4 carbon atoms, 30% to 40% having 5 carbon atoms, along with 10% to 25% of heavier gasoline constituents, said fuel exhibiting the following distillation curve:

10% evaporated between -30° and +30° F.  
50% evaporated between 50° and 100° F.  
90% evaporated between 100° and 170° F.

2. A priming fuel for starting gasoline engines

at low temperatures comprising a liquid mixture of normally gaseous and low boiling paraffinic and olefinic hydrocarbons, 10% to 25% having 3 carbon atoms, 15% to 45% having 4 carbon atoms, 30% to 40% having 5 carbon atoms, along with 10% to 25% of heavier gasoline constituents, said fuel exhibiting the following distillation curve:

10% evaporated between -30° and +30° F.

50% evaporated between 50° and 100° F.

90% evaporated between 100° and 170° F.

WILLIAM J. SWEENEY.

UNITED STATES PATENTS

| Number    | Name            | Date          |
|-----------|-----------------|---------------|
| 1,164,357 | Kaufmann        | Dec. 14, 1915 |
| 1,183,038 | Schlaepfer      | May 16, 1916  |
| 1,344,805 | Brackin         | June 29, 1920 |
| 1,394,921 | McKenzie-Martyn | Oct. 25, 1921 |
| 1,431,518 | Garner          | Oct. 10, 1922 |
| 1,624,139 | Kettering       | Apr. 12, 1927 |
| 1,673,620 | Cunradi         | June 12, 1928 |
| 1,990,499 | Odell           | Feb. 12, 1935 |
| 2,175,743 | Coffman         | Oct. 10, 1939 |
| 2,022,847 | Endres          | Dec. 3, 1945  |

OTHER REFERENCES

REFERENCES CITED

The following references are of record in the file of this patent:

15 Nash and Howes, "Principles of Motor Fuel Preparation and Application" (1935), vol. 1, page 129.